

# United States Patent Office

2,933,379

Patented Apr. 19, 1960

1

2,933,379

## STABILIZED MOTOR FUEL

Ellis K. Fields, Chicago, Ill., and Allen E. Brehm, Griffith, Ind., assignors to Standard Oil Company, Chicago, Ill., a corporation of Indiana

No Drawing. Application January 16, 1958  
Serial No. 709,195

7 Claims. (Cl. 44—63)

The present invention relates to new and useful compositions of matter, and particularly to stabilized light hydrocarbon distillate fuels and to the method of stabilizing such materials against oxidative deterioration in the presence of metals or metal compounds which catalyze such oxidation, for example copper, vanadium, manganese, cobalt, chromium and the like, and compounds thereof. More particularly, the invention is directed to stabilized hydrocarbon motor fuels and to the method of stabilizing petroleum products.

Petroleum products, for example motor fuels, naphthas, Diesel fuels, fuel oils, etc. are susceptible to oxidative deterioration, particularly in the presence of metals which are oxidation catalysts, for example copper, vanadium, cobalt, chromium, etc. and compounds thereof.

An example of such oxidative deterioration is the formation of gum and/or color in storage or in use of certain types of motor fuels, particularly those obtained from cracking processes. In order to inhibit such gum and/or color formation, it has been common practice to add to such fuels various types of anti-oxidants such as for example aminophenols, substituted aminophenols, naphthols, aromatic hydroxy compounds, hard wood tar distillates, and other known anti-oxidants. It has been observed that when motor fuels containing anti-oxidants are stored in metal containers or come in contact with metal surfaces containing copper or copper alloys, the inhibiting effect of the anti-oxidant is decreased to the point where gum forms in such fuels in spite of any anti-oxidant they may contain. This deterioration of anti-oxidants is also encountered in fuels which have been subjected to the copper chloride sweetening process.

It is an object of the present invention to provide light hydrocarbon distillate fuels resistant to oxidative deterioration. Another object of the invention is to provide a method of inhibiting the oxidative deterioration of light hydrocarbon distillate fuels in the presence of metals or metal compounds which are oxidation catalysts. Still another object of the invention is to provide hydrocarbon motor fuels which are resistant to oxidative deterioration. A further object of the invention is to provide a method of inhibiting the oxidative deterioration of gasoline containing, or coming in contact with, metals or metal compounds, which catalyze such oxidative deterioration. Other objects and advantages of the invention will become apparent from the following description thereof.

We have discovered that the foregoing objects can be attained by incorporating in light hydrocarbon distillate fuels, normally susceptible to oxidative deterioration, a small but inhibiting amount, for example, from about 0.0001% to about 1.0%, preferably from about 0.003%

2

to about 0.05% of an 8-hydroxy quinoline derivative having the general structure



in which R is a tertiary alkyl radical of from about 4 to about 24 carbon atoms.

Compounds of the above structure are readily prepared by heating to a temperature of from about 100° F. to about 220° F., an equal molar mixture of 8-hydroxy quinoline and a tertiary alkyl azomethine. Heating, with stirring, is continued at about 220° F. while blowing the nitrogen for about one hour or until there is no longer the odor of the azomethine. Tertiary alkyl azomethine such as t-butyl-, t-amyl-, t-hexyl-, t-octyl-, t-nonyl, t-dodecyl-, t-octadecyl-, and t-eicosyl-azomethines may be employed.

The preparation of the additive of the present invention is illustrated by the following example:

### EXAMPLE I

A mixture of 28.2 g. t-octyl azomethine (0.2 mole) and 29 g. (0.2 mole) 8-hydroxy quinoline was heated and stirred. At 140° F. all solid has dissolved and reacted. Heating was continued at 220° F. for 1 hour with N<sub>2</sub> blowing. All the odor of the azomethine had disappeared. The product, 57 g.,



is a viscous orange-brown liquid. Anal.: Calcd. for C<sub>18</sub>H<sub>25</sub>N<sub>2</sub>O: N, 9.82%. Found: N, 9.69%.

The effectiveness of the above described additive in inhibiting oxidative deterioration, as indicated by an increase in the induction period of a gasoline, determined by the ASTM D-525 Induction Period Test is demonstrated by the data in Table I.

Table I

| Sample No. | Composition                                              | Induction Period, Mins. |
|------------|----------------------------------------------------------|-------------------------|
| A          | Gasoline No. 1                                           | 390                     |
| B          | A+3 lb. product of Example I per 1,000 bbls. (0.0009%).  | 435                     |
| C          | A+1 p.p.m. Copper (Acetate)                              | 145                     |
| D          | C+1 lb. product of Example I per 1,000 bbls. (0.0003%).  | 255                     |
| E          | Gasoline No. 2+1 p.p.m. Copper (Acetate)                 | 95                      |
| F          | E+1 lb. product of Example I per 1,000 bbls. (0.0003%).  | 130                     |
| G          | E+2 lbs. product of Example I per 1,000 bbls. (0.0006%). | 240                     |

The additives of the present invention are effective in reducing lead deposition resulting from the degradation of tetraethyl lead in gasoline during long periods of storage; leaded gasoline can contain from about 0.5 to about 5.0 milliliters tetraethyl lead per gallon of fuel. This property is demonstrated by the data in Table II which were obtained by storing samples of a gasoline containing 2.5 cc. tetraethyl lead per gallon, with and without additives, for a period of eight months at 110° F.

3  
Table II

|                                                                 | Mg. (1)<br>Insol.<br>Lead/500<br>ml. | Mg. (2)<br>Insol.<br>Organic<br>sediment<br>per<br>500 ml. | Mg. (3)<br>ASTM<br>D-381<br>gum/100<br>ml. | Mg. (4)<br>Total<br>Insolubles<br>and<br>soluble<br>gum per<br>100 ml. |
|-----------------------------------------------------------------|--------------------------------------|------------------------------------------------------------|--------------------------------------------|------------------------------------------------------------------------|
| 1. Control (Average of two)                                     | 5.1                                  | 6.0                                                        | 5.7                                        | 7.9                                                                    |
| 2. +# Additive A* /1,000 bbls.                                  | 2.3                                  | 4.3                                                        | 3.6                                        | 4.9                                                                    |
| 3. +# Product Example I/<br>1,000 bbls.                         | 3.6                                  | 9.4                                                        | 3.9                                        | 6.5                                                                    |
| 4. +# Additive A/1,000 bbls.                                    | 3.5                                  | 6.1                                                        | 5.0                                        | 6.9                                                                    |
| 5. +# Additive A/1,000 bbls.<br>+# Product Ex. I/1,000<br>bbls. | 2.8                                  | 4.8                                                        | 3.3                                        | 4.8                                                                    |

The values of (1), (2), (3) and (4) were obtained by the following procedure. The total contents (500 ml.) of the quart bottle was filtered through a tared fine sintered glass crucible. The filtered gasoline was evaluated for soluble gum by the ASTM D-381 Method. These results are shown in Table II as milligrams ASTM D-381 gum per 100 milliliters. The quart bottle was washed with a mixture of methanol, acetone and chloroform and all of the solids removed. The washings were put through the filter crucible containing the insolubles previously collected, and the effluent collected in a clean receiver. The effluent contained gasoline insoluble organic sediment since this mixture of solvents is excellent for dissolving fuel insoluble oxidation products except for lead compounds. Evaporation of the effluent under conditions of the ASTM D-381 Method gave the milligrams of insoluble organic sediment per 500 milliliters of fuel. These data are shown in Table II. At this point, the tared sintered glass crucible contained only fuel insoluble lead compounds which were determined quantitatively by drying and weighing the crucible. The results are shown in Table II as milligrams of insoluble lead per 500 milliliters. The column headed "Milligrams total insolubles and soluble gum per 100 milliliters" represent the sum of the other three columns converted to a 100 ml. basis where necessary.

\*Additive A is N,N'-di-sec.butyl-p-phenylene diamine marketed as Du Pont Antioxidant No. 22.

The above data demonstrate that the combination of one pound per 1000 barrels gasoline of each of the antioxidant and the additive of the present invention (No. 5) is more effective in inhibiting the degradation of tetraethyl lead and the oxidative deterioration of the hydrocarbon motor fuel than 2-5 pounds of the antioxidant per 1000 barrels of fuel (No. 2 and 4) or 5 pounds of the product of Example I per 1000 barrels of fuel (No. 3).

As noted above, the additives of the present invention are added to light petroleum distillates in small concentrations. However, they can also be handled in the form of concentrates in hydrocarbon distillates, which can be blended back in the finished composition to the desired concentration. The light petroleum distillates are conventionally produced by crude oil fractionation, cracking processes, and special conversion processes such as reforming, alkylation, polymerization, etc. The light distillates have a boiling point of from about 90° F. to about 200° F.; those in the gasoline range boiling from about 100° F. to about 400° F., and those in the diesel fuel and heating oils boiling in the range of from about 350° F. to about 700° F.

Percentages given herein and in the appended claims are by weight unless otherwise stated.

The additive of the present invention can be used in combination with antioxidants, anti-wear agents, agents to inhibit spark-plug fouling, corrosion inhibitors, etc.

While the invention has been described and illustrated by way of preferred embodiments thereof, it will be apparent to those skilled in the art that variations and modifications may be made without departing from the scope of the present invention as defined by the appended claims.

We claim:

1. A stabilized hydrocarbon light distillate composition comprising a major proportion of a light petroleum distillate, normally susceptible to oxidative deterioration

4

and a small but sufficient amount to inhibit such oxidative deterioration, of an 8-hydroxy quinoline derivative having the general structure



5

10 in which R is a tertiary alkyl radical having from about 4 to about 24 carbon atoms.

2. The composition of claim 1 in which R is a tertiary octyl radical.

15 3. The composition of claim 1 in which the weight petroleum distillate is a petroleum motor fuel.

4. A gasoline stabilized against oxidative deterioration containing from about 0.0001% to 0.05% of an 8-hydroxyquinoline derivative having the general structure



25 5 in which R is a tertiary alkyl radical having from about 4 to about 24 carbon atoms.

6. A gasoline stabilized against oxidative deterioration containing from about 0.0001% to about 0.05% of an 8-hydroxyquinoline derivative having the general structure



35

35 7. A hydrocarbon fuel for spark-ignition internal combustion engines comprising a major proportion of a petroleum distillate in the gasoline distillation range, normally susceptible to oxidative deterioration, from about 0.5 to 5.0 milliliters tetraethyl lead per gallon of said distillate, which tetraethyl lead is susceptible to degradation and from about 0.0001% to about 0.05% of an 8-hydroxyquinoline derivative having the general structure



50

in which R is a tertiary alkyl radical of from about 4 to about 24 carbon atoms, whereby said oxidative deterioration of said petroleum distillate and said degradation of the tetraethyl lead is inhibited.

55 8. A hydrocarbon fuel as described in claim 7 in which R is a tertiary octyl radical.

#### References Cited in the file of this patent

#### UNITED STATES PATENTS

- |           |           |               |
|-----------|-----------|---------------|
| 2,030,033 | McConnell | Feb. 4, 1936  |
| 2,136,788 | Fairlee   | Nov. 15, 1938 |
| 2,198,961 | Dietrich  | Apr. 30, 1940 |
| 2,372,588 | Larsen    | Mar. 27, 1945 |
| 2,647,824 | Jones     | Aug. 4, 1953  |
| 2,861,975 | Thompson  | Nov. 25, 1958 |